

Aug. 27, 1929.

J. H. WHITE

1,725,773

ELECTRIC CONDUCTOR

Filed Nov. 19, 1924

2 Sheets-Sheet 1



Fig. 2



Fig. 3



Inventor:  
John H. White,  
by *John H. White* Atty

Aug. 27, 1929.

J. H. WHITE

1,725,773

## ELECTRIC CONDUCTOR

Filed Nov. 19, 1924

2 Sheets-Sheet 2



## UNITED STATES PATENT OFFICE.

JOHN H. WHITE, OF CRANFORD, NEW JERSEY, ASSIGNOR TO WESTERN ELECTRIC COMPANY, INCORPORATED, OF NEW YORK, N. Y., A CORPORATION OF NEW YORK.

## ELECTRIC CONDUCTOR.

Application filed November 19, 1924. Serial No. 750,718.

This invention relates to electric conductors, and particularly to flexible conductors and cables.

The invention is especially applicable to 5 telephone switchboard cable and distributing frame wire which are used extensively in telephone exchanges.

It is the object of this invention to produce an economical and efficient insulated conductor particularly suitable for indoor use such 10 as is encountered in and around telephone switchboards and associated distributing equipment of a telephone exchange.

The mechanical and electrical requirements of telephone switchboard cable are very 15 severe. From a mechanical standpoint, the cable must be flexible enough for use in a telephone exchange, for example to allow frequent bending and twisting, as well as to 20 permit a group of cables to be wedged apart for the purpose of making necessary electrical connections.

From an electrical standpoint, the individual conductors must be far enough apart 25 to keep down the capacity, and the pairs of conductors constituting a circuit must be twisted in order to avoid cross-talk. Most important of all, perhaps, the insulation resistance of the individual conductors must 30 be high.

It is well known that different insulating materials vary widely in their electrical insulation resistance properties. Fibrous materials such as cotton and tussah floss silk, 35 possess good insulation resistance properties when dry, but it is found that when these materials are exposed to moist air their insulation resistance is considerably lowered. Regardless of their relative insulating properties, the insulation resistance of all such materials falls off rapidly under rising humidity 40 conditions.

There is a distinction between the requirements of a moisture-proof switchboard cable 45 and a water-proof cable such as is used for under-water signaling. The atmospheric conditions of a telephone exchange may approach, but never reach the dew point. The switchboard cable in a telephone exchange, 50 while never submerged in water, is at all times subject to the deleterious action of moisture in the air which is always present in varying amounts, depending upon climatic and humidity conditions.

55 Furthermore, since telephone switchboard

cables in use are always carrying some current through some of the conductors, the cable is at all times slightly warmer than the room temperature and hence never below the dew point even during a rainstorm. 60

While the amount of water absorption is not necessarily a direct and proportionate measure of the insulation resistance of fibrous insulating materials, nevertheless the presence of water in all cases produces a deleterious 65 effect upon the insulation resistance properties. The presence of water in a switchboard cable establishes short-circuit paths between the various conductors, thus destroying their efficiency for purposes of telephonic communication, and also sets up an electrolytic action 70 which decomposes the conductors and ultimately renders the cable unfit for service.

Since it is inexpedient for mechanical reasons to cover a switchboard cable with a 75 hermetically impervious sheath, it will be seen that the ability of the cable to resist the action of moist air must be high.

A switchboard cable which has been used successfully under medium humidity conditions 80 consists of a plurality of black enamel covered conductors each having one, two or even three wrappings of floss silk, these conductors being twisted in pairs and assembled in layers with interleaving hard paper strips, 85 forming a compact pliable group of conductors. Such a group of conductors is then overwound with tapes of cloth, tinfoil and a braided covering which is painted, preferably with fireproof paint. 90

Although dry floss silk possesses excellent properties of insulation resistance, it will be seen from the above that elaborate precautions are taken to minimize the effect of moisture which would tend to reduce its insulation resistance. The enamel coating is employed to assist in excluding moisture, but does not of itself render the conductor moisture-proof since commercial enamel wire frequently contains pinholes or gaps which are 95 formed either during the coating process or by cracking the enamel by bending or twisting the wire.

Such cables, however, are open to several important objections, such as the difficulty of 100 soldering the enameled wire and the high cost and limited supply of floss silk. Furthermore, even with all the above precautions taken, under extreme humidity conditions, such as are encountered in the tropics, the 110

action of moisture has been found to injure the cable in a comparatively short time.

This invention overcomes the difficulties outlined above by providing a cheap and efficient switchboard cable, the insulation resistance of which remains substantially unaffected by all humidity conditions below the dew point.

In accordance with one of its features, the invention provides a new and improved method of treating the individual conductors of a switchboard cable, in which the use of an enamel coating may be eliminated and in which cotton insulation is employed in place of the more expensive floss silk.

Briefly, this is accomplished by converting the rather hygroscopic cotton into such a condition that its insulation resistance is substantially unaffected by moist air. The cotton insulation upon the conductor is first treated to expel moisture and is then thoroughly impregnated with a solution of cellulose acetate which is free from electrolytic and hygroscopic materials.

The result of the process is to produce a conductor provided with a glossy tube-like cover in which the cotton fibres are enclosed in a solid matrix of cellulose acetate. This insulating cover retains a high insulation resistance under substantially all humidity conditions up to the dew point.

Although the cotton insulation is somewhat repellent to the cellulose acetate solution, the impregnating process is hastened and rendered more thorough by first treating the insulation with a priming agent designed to eliminate all air pockets and to facilitate the entrance of the cellulose acetate solution into the pores and interstices of the insulation.

In the preferred form of the invention, the priming agent consists of a solvent of cellulose acetate, such as acetone. The insulated conductor so treated is next dried off to such a point that while insufficient liquid acetone is left in the fibres to disadvantageously dilute the cellulose acetate solution which is subsequently applied, still sufficient acetone vapor is left in the cotton insulation to displace the air.

This operation may be performed in such a way that the amount of acetone vapor left in the insulation is such that the unavoidable evaporation of the solvent, such as acetone, from the cellulose acetate solution is made up by the acetone carried thereto in the insulation, so that the cellulose acetate solution grows neither thinner or thicker.

The impregnating bath consists of a solution of chemically pure cellulose acetate dissolved in highly refined acetone, both of which are entirely free from hygroscopic and electrolytic materials. After a thorough impregnation, the insulated conductor is passed through a current of hot air, thus

hastening the evaporation of the acetone and leaving the conductor when dry with a smooth and glossy cover in which the fibres of insulation are enclosed in a matrix of cellulose acetate. The depth to which the insulation is impregnated may vary as desired.

It has previously been proposed to enamel bare conductors with cellulose acetate lacquers, as well as to treat fabrics with cellulose acetate in order to produce a glossy finish. While cellulose acetate has been used in the electrical arts, it has heretofore proved of negligible value except as a varnish.

Conductors coated with cellulose acetate lacquers are entirely unsuited for use in telephone switchboard cable because such a coating is easily chipped off when the conductor is bent or twisted. Furthermore, the cellulose acetate heretofore employed has always contained various deleterious substances which tend to attract moisture, and previously known methods of treating electrical apparatus have not been such as to increase the moisture resisting qualities of the insulation.

The various features and advantages of the invention are described in detail with reference to the accompanying drawing, in which:

Figure 1 is a sectional view illustrating the method of treating an insulated conductor in accordance with the invention.

Figure 2 is a plan view illustrating two portions of an insulated conductor, one of which is untreated and the other of which is treated in accordance with the invention.

Figure 3 is a sectional view of a switchboard cable constructed in accordance with the invention.

Figure 4 shows a series of curves illustrating the efficiency of telephone conductors insulated in accordance with the invention.

As shown in Fig. 1, a conductor insulated with cotton or other suitable insulating material is drawn from a supply reel 5 to an impregnating tank 6 containing acetone. From the tank 6, the conductor passes through a channel or chamber 7 to an impregnating tank 8 containing the cellulose acetate bath. The conductor is then drawn from the tank 8 through a drying chamber 9 to a suitable take-up reel 10.

The insulated conductor on the reel 5 is heated to remove all moisture before the impregnating process. Any number of layers of fibre insulation may be employed. For example, the conductor may be insulated with a single layer of cotton yarn of sufficient coarseness to secure the desired separation between the conductors of the cable to keep down the capacity therebetween. It is also preferable to use cotton yarn that is naturally as little hygroscopic as possible, avoiding the use of cotton that has been bleached or otherwise treated in such a way as to increase its hygroscopic properties. Either be-

fore or after being spun into yarn, the cotton may be tested and if found to contain soluble hygroscopic and saline materials, it may be put through an exhaustive treatment of pure 5 hot water to remove such materials.

The tank 6 is provided with a tightly fitting cover 11 and the tank 8 is provided with a similar cover 12 to prevent the entrance of moisture thereto. The chamber 7 is tightly 10 fastened at one end to the tank 6 and at the other end to the tank 8 to prevent the entrance of moisture thereto. The drying chamber 9 is similarly fixed to the cover 12 of the tank 8, thereby providing a continuous 15 air-free passage for the insulated conductor during the entire process.

The insulated conductor is drawn from the reel 5 through a small hole or vent 13 in the tank 6. The vent 13 is preferably just large 20 enough to permit the passage of the conductor, and if desired may be filled with a suitable stuffing material as an added precaution against the entrance of moisture to the tank. The tank 6 contains a bath of highly refined 25 acetone, free from moisture and electrolytic and hygroscopic materials. The conductor is passed through the acetone over suitable guide rollers at such a rate as to allow the acetone to thoroughly impregnate the fibers 30 of the insulation.

The insulated conductor impregnated with acetone is passed from the tank 6 through the chamber 7 to the impregnating tank 8. A strong current of hot dry air from an inlet 35 supply pipe 14 is circulated through the chamber 7 to an outlet pipe 15 to hasten the evaporation of the liquid acetone contained in the insulation. The hot dry air is preferably maintained at about the temperature of the 40 boiling point of acetone.

The passage of the conductor through the chamber 7 is preferably so regulated that the insulation will be dried to such a point that while insufficient liquid acetone is left 45 in the insulation to disadvantageously dilute the cellulose acetate solution contained in the tank 8, still sufficient acetone vapor is left in the pores and interstices of the insulation to displace the air, and also to compensate for 50 the unavoidable evaporation of the solvent contained in the tank 8. The degree of evaporation may be controlled in several ways, such as by properly gauging the length of the chamber 7, or by regulating the temperature 55 and velocity of the hot dry air, and by regulating the speed at which the conductor is drawn through the chamber 7.

The hot air containing the acetone vapor liberated in the chamber 7 is drawn off 60 through the outlet pipe 15 to a suitable condensing apparatus (not shown) where the acetone is reclaimed, and returned to the tank 6 for further use. The exclusion of damp or other air from the tanks 6 and 8 prevents 65 a film or skin from forming on the top of

the solutions contained therein, since the atmosphere above the free surface of the solution in these tanks is saturated with pure acetone vapor.

The insulated conductor treated in the 70 chamber 7 in the manner described above is drawn through the impregnating tank 8 containing the cellulose acetate bath. Great care is taken in the preparation of this solution. A water washed cellulose acetate pulp is first 75 prepared, which is so thoroughly free from any residual hygroscopic and electrolytic saline or other matter, such as sulphuric acid and zinc chloride which may have been used as catalytic agents in preparing the cellulose 80 acetate, that when a sample is exhaustively extracted with water in an extraction apparatus, the water shows no reaction with barium chloride or silver nitrate. The pulp is then dried, preferably at not more than a 85 few degrees above the temperature of boiling water until samples taken show constant weight. The cellulose acetate solution is then prepared by dissolving about 150 grams to 300 grams of the dry pulp to the United 90 States gallon of highly refined acetone of specific gravity of .797 at 60° Farenheit. This solution is allowed to settle and the clear supernatant liquor is drawn off for use in the 95 impregnating tank 8, while the gray undissolved sludge, if such remains, is rejected.

The insulated conductor is passed through the tank 8 containing the cellulose acetate solution prepared in the manner described above, over suitable guide rollers, and becomes 100 thoroughly impregnated with the solution.

The impregnated conductor emerges from the tank 8 through a small vent 16 in the airtight cover 12 into the drying chamber 9. If desired, the vent 16 may contain a wiper or 105 scraper for removing the excess solution which clings to the insulation. A strong current of hot dry air is circulated through the chamber 9 from an inlet pipe 17 which may be associated with the same source of 110 supply as the inlet pipe 14 in the chamber 7, to an outlet pipe 18 which may be associated with the same condensing apparatus (not shown) to which the outlet pipe 15 is connected. The hot dry air is preferably maintained at the temperature of the boiling point of acetone, and the temperature may be observed at all times by means of a thermometer 115 19 associated with the inlet pipe 17.

The acetone contained in the insulation is 120 rapidly evaporated in the chamber 9, leaving a glossy coating upon the insulation. The conductor is drawn over a suitable guide roller through a vent 20 in the chamber 9 to the take-up reel 10. A scraper or smoothing 125 die may be mounted on the inner wall of chamber 9, for example at the vent 20 for the purpose of removing uneven particles of cellulose acetate which may tend to cling to the surface of the insulation, thus giving a smooth 130

and polished appearance to the conductor. The exact point in the drying chamber to place the die is obtained by trial.

Ordinarily, in treating fibrous materials with cellulose acetate, it is very difficult to obtain a thorough penetration of the cellulose acetate solution into the inner pores and interstices of the material. This is primarily due to the fact that the fibrous materials are naturally repellent to the rather thick cellulose acetate solution, and also because the cellulose acetate solution does not readily displace the air in the lower layers of the fibrous material. It has been found, however, that when an insulated conductor is first impregnated with a solvent such as acetone used in the preparation of the cellulose acetate solution, and the conductor so treated is then freed of the liquid solvent to such an extent that only a portion of the vapor remains, and is then immersed in a pure cellulose acetate solution, the insulated conductor is thoroughly impregnated down to the wire and the flaws heretofore encountered are entirely obviated.

The evaporation of the acetone in the chamber 9 leaves a moisture resisting insulated cover upon the wire in which the fibres of insulation are enclosed in a matrix of solid cellulose acetate. The cellulose acetate, in drying, causes a shrinking down of the fibres and produces a solid tube-like insulation which is considerably smaller in diameter than the original unimpregnated loose insulation. This is illustrated more clearly in Fig. 2 which is a copy of an actual photograph showing a portion 21 of a cotton covered wire which is unimpregnated and a portion 22 of the same conductor impregnated in accordance with the invention. It will be seen that the impregnating process has materially reduced the space occupied by the insulation in the conductor 22, thereby permitting a greater bulk of conductors to be enclosed in a given space in a switchboard cable, when capacity considerations admit of it.

Fig. 3 shows a switchboard cable prepared in accordance with the invention. This cable consists of a plurality of copper conductors 23, which may if desired be tinned to facilitate soldering operations. The conductors 23 are each covered with one or more layers of cotton insulation 24 impregnated with cellulose acetate in the manner described above. The insulated conductors are twisted in pairs and the bundle grouped together by means of a serving of cotton yarn 25 and a spirally served paper strip 26, and are overwound with a fabric tape 27 and a braided fabric cover 28. If desired, the outer cover 28 may be covered with a coat of fire-proof paint. Other and different covering materials may also be employed.

The outer cover 28 may also be impregnated with cellulose acetate in the manner described above to further increase the moisture resisting quality of the cable. This precaution may be desirable where the cable is to be used in localities where extremely high humidity conditions prevail.

Exhaustive tests have been made which illustrate the efficiency of an insulated conductor prepared in the manner described above. The table given below illustrates the average results of prolonged tests made in connection with cellulose acetate impregnated cotton covered wire, untreated cotton covered wire and untreated tussah silk floss covered wire under varying humidity conditions. These tests were conducted in a humidity room maintained at a constant temperature of 85° Fahrenheit. The humidity, however, was varied at times from day to day, and at times was maintained constant for two or more days, and the electrical tests were made after the three samples of conductor had been subjected to the same given humidity conditions for at least 24 hours. The figures represent the insulation resistance in megohms per fifty feet of No. 22 B. & S. gauge conductor.

Insulation resistance—Megohms per 50 feet of conductor.

| Insulation                       | First day H. 65% |            | Second day H. 75% |            | Third day H. 85% |            | Fourth day H. 90% |            | Eighth day H. 65% |            | Ninth day H. 75% |            | Tenth day H. 85% |            | Eleventh day H. 90% |            | Twelfth day H. 85% |            | Thirteenth day H. 75% |            | Fifteenth day H. 65% |            | Sixteenth day H. 85% |            | Seventeenth day H. 90% |            | Eighteenth day H. 85% |            | Nineteenth day H. 90% |            | Twentieth day H. 80% |            | Twenty-first day H. 90% |  |
|----------------------------------|------------------|------------|-------------------|------------|------------------|------------|-------------------|------------|-------------------|------------|------------------|------------|------------------|------------|---------------------|------------|--------------------|------------|-----------------------|------------|----------------------|------------|----------------------|------------|------------------------|------------|-----------------------|------------|-----------------------|------------|----------------------|------------|-------------------------|--|
|                                  | First day        | Second day | First day         | Second day | First day        | Second day | First day         | Second day | First day         | Second day | First day        | Second day | First day        | Second day | First day           | Second day | First day          | Second day | First day             | Second day | First day            | Second day | First day            | Second day | First day              | Second day | First day             | Second day | First day             | Second day | First day            | Second day |                         |  |
| Cellulose acetate cotton.....    | 118.5            | 23.6       | 2.02              | .352       | 58.8             | 14.4       | 0                 | 1.25       | .518              | .856       | 4.73             | 19.8       | 31.5             | 0          | .548                | .325       | .279               | .221       | .111                  |            |                      |            |                      |            |                        |            |                       |            |                       |            |                      |            |                         |  |
| Untreated cotton.....            | .373             | .093       | .009              | .004       | .200             | .068       | 0                 | .018       | .006              | .006       | .011             | .038       | .112             | .136       | 0                   | .010       | .007               | .004       | .002                  |            |                      |            |                      |            |                        |            |                       |            |                       |            |                      |            |                         |  |
| Untreated Tussah silk floss..... | 119.3            | 13.2       | .246              | .021       | 14.4             | 1.89       | 0                 | .018       | .008              | .024       | .181             | 1.39       | 2.37             |            | .011                | .003       | .004               | .001       | .003                  |            |                      |            |                      |            |                        |            |                       |            |                       |            |                      |            |                         |  |

From the above table it will be seen that the insulation resistance of the conductor prepared in accordance with the invention is much superior to that of the untreated cotton covered conductor or the untreated tussah silk floss covered conductor under varying humidity conditions. While the insulation

resistance of the silk floss covered conductor is slightly higher than the insulation resistance of the cellulose acetate cotton covered conductor, after being subjected to a relative humidity of 65% on the first day, it will be noted that this condition is reversed at the end of the second day when both conductors

have been subjected to a relative humidity of 75%. On the third and fourth days, after being subjected to humidity conditions of 85% and 90%, the insulation resistance of the 5 conductor prepared in accordance with the invention is much higher than that of either the untreated cotton covered conductor or the untreated silk floss conductor. On the fifth day, the humidity was dropped from 90% to 10 65% to determine the manner in which the several conductors would recover from the effects of the extremely high humidity to which they were subjected on the fourth day. The results, as may be seen from the table, 15 indicate the vastly superior qualities of the cellulose acetate impregnated cotton insulation. The varying humidity conditions to which the several conductors were subjected throughout the test, while severe, nevertheless 20 indicate the conditions to which the switchboard cable may be subjected under actual operating conditions.

The efficiency of switchboard cable made of conductors prepared in accordance with the 25 invention for purposes of telephonic communication is illustrated graphically in Fig. 4. Such cables must have a low leakage from wire to wire, which may be expressed as a conductance, for the efficient transmission of 30 speech, otherwise the voice currents would be greatly attenuated by such short circuiting type of wire-to-wire leakage during transmission. Fig. 4 represents such leakage measure as a conductance in micromhos per fifty feet 35 of a pair of No. 22 B. & S. gauge conductors at 1,000 cycles per second, which frequency represents practical operating conditions. The curve "H" represents the humidity to which the conductors were subjected from 40 day to day over a period of several weeks. The curve 1 represents the leakage between the untreated cotton insulated conductors, while curve 2 represents the leakage between the untreated tussah silk floss insulated conductors, and the curve 3 represents leakage 45 between the cellulose acetate impregnated cotton covered conductors constructed in accordance with the invention. It will be seen that the leakage of the cotton insulated conductors increases rapidly with the relative 50 humidity, rendering the conductors highly inefficient for purposes of telephonic communication under humidity conditions which are encountered in ordinary telephone practice. The leakage of the silk floss covered conductors likewise increases rapidly under rising humidity conditions, although to a somewhat less extent than the cotton covered conductors. The curve 3 indicates, however,

that the leakage of the cellulose acetate impregnated cotton covered conductors constructed in accordance with the invention, varies unappreciably under substantially all humidity conditions below the dew point.

It will be seen from the above that the 65 electrical characteristics of conductors prepared in accordance with this invention are materially improved, and that a switchboard cable prepared in this manner may be operated efficiently under all conditions of operation which are encountered in a telephone exchange.

A particular advantage of the invention is the conversion of the cotton, which is cheap but which possesses a poor insulation resistance, in moist air into a condition such that it has a higher insulation resistance in moist air than the more expensive silk which has heretofore been employed in the manufacture 75 of switchboard cables.

While the invention has been described with particular reference to cotton covered conductors, it is to be understood that it is 80 equally applicable to conductors insulated with other materials.

The invention is also capable of other modifications and adaptations not specifically referred to but included within the scope of the appended claims.

What is claimed is:

1. An electrical conductor having a non-water-proof insulating covering which retains its insulating qualities under conditions where it is always warmer than the dewpoint of the surrounding air, characterized by the provision of an impregnating material containing a solid ester dissolved in a plastic solvent and free from electrolytic materials.

2. An electrical conductor having a non-water-proof insulating covering which retains its insulating qualities under conditions where it is always warmer than the dewpoint of the surrounding air, characterized by the provision of an impregnating material containing a cellulose ester and free from hydroscopic and electrolytic materials.

3. An electrical conductor having a non-water-proof insulating covering which retains its insulating qualities under conditions where it is always warmer than the dewpoint of the surrounding air, characterized by the provision of a cotton serving impregnated with cellulose acetate free from hydroscopic and electrolytic materials.

In witness whereof, I hereunto subscribe my name this 14th day of November A. D., 1924.

JOHN H. WHITE.